

## UNITED STATES PATENT OFFICE

JAMES B. GREAGLE, OF BALTIMORE, MARYLAND, ASSIGNEE OF ONE-HALF TO  
WILLIAM W. VARNEY, OF BALTIMORE, MARYLAND

## NONFERROUS ALLOY

No Drawing.

Application filed October 17, 1929. Serial No. 400,448.

- The object of my new alloy is the production of a non-ferrous alloy having metallic properties generally, but which is free from attack from many acids, alkalis and gases. 5
- 6 A further object of my invention is the production of a non-ferrous alloy which is particularly free from attack by hydro-chloric, nitric, or sulphuric acids, or aqua regia.
- 10 10 A further object of my invention is the production of a non-ferrous alloy which is free from attack by ammonia chloride, chlorine, ammonia, mine waters and alkalis generally.
- 15 15 A further object of my invention is the producing of a non-ferrous alloy which is free from attack by sulphurous fumes and gases evolved in the production or refining and manufacturing of oils and gasoline, and 20 free from attack by hypo-chlorides and hyposulphites.
- A further object of my invention is a new process of alloying the elements herein mentioned.
- 25 25 A further object of my invention is a new process for obtaining the elements and compounds herein mentioned.
- A further object of my invention is a new process of separating tantalum and niobium.
- 30 30 A further object of my invention is a new process of obtaining uranic acid.
- A further object of my invention is a new process of obtaining niobic acid.
- 35 35 A further object of my invention, is a new process of obtaining yttric acid.
- With the foregoing and other objects in view, my invention consists of the methods employed, combination and arrangement of systems and means as hereinafter specifically provided, but it is understood that changes, variations and modifications may be resorted to which come within the scope of the claims hereunto appended.
- 40 40 Broadly, my new non-ferrous alloy comprises tantalum, yttrium, uranium and niobium. And it is preferably for certain uses that the tantalum content be of relatively high proportion to the niobium and uranium content, and that the yttrium content be of 45 50 relatively low proportion to the tantalum and niobium content.
- As a concrete example, which I have found gives a very satisfactory non-ferrous alloy for the purposes indicated, the tantalum content varies within the range of 30-50%, the niobium content varies from 12-26%, the 55 yttrium content varies from 8-12%, and the uranium content varies from 8-12%. I have found that it is preferable to have the tantalum content equal the combined content of the niobium, yttrium and uranium. 60
- In the preparation of my alloy I have found it desirable to add the tantalum content after the other contents are fused, and 65 that the tantalum content must be free from iron and other impurities.
- In the making up of this alloy, which is formed by taking ingredients embodying the above metals, or elements, respectively, in 70 metallic form and heating the mixture, the metal content of the metals suggested; namely, tantalum, yttrium, niobium and uranium, are merged into an alloy.
- One example of forming this alloy is by 75 taking the commercially pure metals in the proportions as above named and melting the same to obtain an intermixed molten mass which when properly done and upon cooling will yield a solid alloy of the above analysis. 80 This alloy appears as a grayish-white, ductile metal, a good conductor of heat and electricity proportioned to the tensile strength of ordinary machine steel; and I have further found if it is cast in a closed mold, will be 85 soft, or if cast in an open or chilled mold, will be hard, and will melt at practically 2700 degrees C. This temperature, however, is only suggestive, as quite a range of melting temperature may be obtained depending upon 90 the various percentages of mix, likewise, its relative hardness and ductility.
- This alloy, as above, possesses metallic properties, but is substantially free from attack by hydro-chloric, nitric and sulphuric acid, or gases. The alloy is also free from attack by sulphurous fumes, salt water or air, chlorine, and the gases created in distilling and refining crude petroleum and other 95 mineral oils. 100

The alloy is also free from attack by calcium and other chemical hypo-chlorides, and by sodium and potassium hypo-chlorides, and by sodium and other chemical hypo-sulphites.

The physical and chemical properties of this alloy, render it especially adaptable for electrode and structural parts of radio tubes. These desirable properties include softness and ease in forming, combined with adequate strength and rigidity, and extremely high melting point.

The alloy, in addition, acts as a getter due to its gas absorption properties above a white heat and may be used alone as a clean-up agent, or in conjunction with a more common agent such as is used to-day, principally magnesium. This makes it particularly important to manufacturers of alternating current radio tubes.

When the alloy is used as a "getter", it may be welded, brazed, or soldered to the plate or structural part of the tube, a much more uniform run of tubes with a smaller percentage of rejection is to be expected when this alloy is used as a getter, or as an accessory to the usual "getter".

This alloy may be readily welded or brazed to such metal as copper, nickel, chromium, etc., which are used in the structural parts of tubes, as it does not oxidize in the air, electric or spot welding is desirable and may be performed without loss or injury to the metal.

It is not acted upon by the following acids or chemicals:

5 Sulphuric acid dilute, or concentrated, hot or cold; nitric acid dilute, or concentrated, hot or cold; hydrochloric acid dilute, or concentrated, hot or cold; aqua regia dilute, or concentrated, hot or cold; hydrofluoric acid dilute, or concentrated, hot or cold; formic acid, concentrated or diluted; oxalic acid, concentrated or diluted; phosphoric acid, concentrated or diluted; carbolic acid, concentrated or diluted; citric acid, concentrated or diluted; tannic acid, concentrated or diluted; sodium acetate 20% solution; iodine acetate 10% solution; chlorine solution, no action; sodium hydroxite, dilute solution; potassium hydroxite, 10%; salt water, no action; sea air, no action; sulphurous atmosphere, no action; carbon monoxide, no action.

In the commercializing of my process herein set forth, I have discovered that tantalum and niobium under commercial working are not inseparable from each other in the ores containing the two elements, notwithstanding the common belief to the contrary; and, further, I have discovered, contrary to the common belief, that the two elements combined are practically alloyable with the other elements herein suggested, and that I do not have to alloy these elements in a separated form as has heretofore been considered absolutely essential.

As a further concrete example of my process of manufacture, I obtain all of the above metals from the mineral known as samarskite.

In order to have my metals in form to be properly alloyed in proportions desired, I obtain or separate them as follows:

My tantalum I obtain as follows: The ore is roasted with  $K_2FL_6$ , four parts to one part of ore until thoroughly fused, poured onto a transite plate, ground to powder and heated with water made slightly acid with HF. Upon cooling, tantalum and niobium separate out by crystallization, re-crystallized again, dissolved as before adding a little potassium carbonate, evaporating to dryness, heating carefully, adding water and boiling the solution. The tantalum separates completely as oxy-fluotantalate

85



While all the niobium remains in solution as oxyfluoniobate ( $K_2NbF_6O$ ).

I obtain my niobium as follows: From the filtrate the niobium is precipitated as niobic acid by evaporating to fuming with sulphuric acid, diluting, washing alkaline with ammonium hydroxide, and re-acidifying with sulphuric acid boiling and precipitating with ammonia.

95

I obtain my yttrium as follows: The ore is pulverized, washed, digested with concentrated HCl to remove the iron, mixed with twice its weight of  $NaCO_3$ , and heated to a white heat. The melt is leached with water and the insoluble residue treated with excess of  $H_2SO_4$  which excess is later driven off. The yttrium sulphate is dissolved in water, precipitated by  $NH_4OH$  and the yttrium hydroxide precipitated as oxide.

100

Uranium: The ore is roasted with an alkali until thoroughly fused, washed with hot water until free of iron and dissolved with  $HNO_3$ . Evaporate the  $HNO_3$  solution obtained to a volume of about 40% and cool. Made neutral with  $NH_4OH$ , add about 5% of  $HC_2H_3O_2$  and 15% of  $HPO_4$ , heat the mixture to boiling, a white precipitate of uranium is formed. Cool to coagulate the precipitate, wash and ignite to  $U_3O_8$ .

110

The most preferred form of the alloy consists of a tantalum content greater than the sum of the niobium and yttrium contents, the yttrium and uranium contents being substantially equivalent. The niobium content being less than the tantalum content and greater than the combined yttrium and uranium content.

115

The alloy possesses metallic properties but is substantially free from attack by hydrochloric, nitric, sulphuric acids or gases. The alloy is free from attack by sulphurous fumes, salt water or air, chlorine and the gases created in the distilling and refining of crude petroleum and other mineral oils.

125

130

The alloy is also free from attack by calcium and other commercial hypo-chlorites and by sodium and potassium hypo-chlorites and by sodium and other commercial hypo-sulphites.

5 Niobium and tantalum are recognized as almost similar elements in their behavior, except their melting point is different, and I take advantage of that in the forming of  
10 my alloy; I take the oxide of the two elements and reduce the niobium first, which attacks the oxide of tantalum, reducing the same.

15 In this specification and claims, when I use the term, "niobic acid", I mean a chemical combination of niobium in any chemical compound; and when I use the term, "tantallic acid", I mean a chemical combination of tantalum in any chemical compound.

20 Attention is especially called to my process described herein where I am enabled to obtain uranium as a precipitate without a precipitating agent, wherein concentration, heating and cooling is availed of whereby a coagulation is obtained, and the elements ordinarily precipitated with the uranium are held in solution.

25 Having thus described my invention, what I claim and desire to secure by Letters Patent is:

30 1. An alloy consisting of tantalum in the proportion of from 30 to 50%, of niobium in the proportion of from 12 to 26%, of yttrium in the proportion of from 8 to 12%, and of uranium in the proportion of from 8 to 12%.

35 2. An alloy of tantalum in the proportion of from 30 to 60%, yttrium and uranium in substantially equal proportion to one another, and of niobium of from 12 to 26%, the combined aforesaid proportions totalling 100%.

40 JAMES B. GRENAGLE.